

H. 20 - C

לענין

3

June 7, 1949.

Filed Feb. 16, 1945

**J. S. PEAKE**  
**MECHANICAL METHOD FOR GRAIN**  
**REFINING MAGNESIUM ALLOYS**

2,472,757

2 Sheets-Sheet 1



Fig. 1



Fig. 2

INVENTOR.  
*John S. Peake*

BY

*Griswold & Burdick*  
ATTORNEYS

June 7, 1949.

Filed Feb. 16, 1945

**J. S. PEAKE**  
**MECHANICAL METHOD FOR GRAIN**  
**REFINING MAGNESIUM ALLOYS**

**2,472,757**

2 Sheets-Sheet 2



Fig. 3



Fig. 4



Fig. 5



Fig. 6



Fig. 7



Fig. 8

INVENTOR.  
John S. Peake

BY

Griswold & Burdick  
ATTORNEYS

## UNITED STATES PATENT OFFICE

2,472,757

## MECHANICAL METHOD FOR GRAIN REFINING MAGNESIUM ALLOYS

John S. Peake, Midland, Mich., assignor to The Dow Chemical Company, Midland, Mich., a corporation of Delaware

Application February 16, 1945, Serial No. 578,254

6 Claims. (Cl. 75—67)

1

The invention relates to a method for treating molten magnesium-base alloys prior to casting. It more particularly concerns a method for treating the molten metal prior to casting whereby reduced grain size and enhanced physical properties are secured in the cast metal.

It is known that in a general way, the finer the grain size of the cast metal the better the tensile strength and related concomitant properties. It is also known that the thermal history of the metal in the molten state has some effect on the grain size of the cast metal. It has been found, for example, that by superheating the molten metal to at least 1472° F., i. e. 392 Fahrenheit degrees or more above the melting point (a temperature between 1600° F. and 1700° F. is usually employed), after the operation of purification by puddling the metal under a suitable flux before casting, the grain size of castings made therefrom is markedly smaller than that of castings of non-superheated metal and the mechanical properties are improved.

This procedure of superheating before casting, as a method of reducing grain size and improving properties, has certain disadvantages which leave much to be desired. Some of these are that the relatively high temperature to which the molten metal must be subjected to produce a given degree of grain size reduction promotes oxidation of metal and consumption of flux, if used, and the life of the melting equipment is shortened due to the more rapid deterioration which occurs at the higher temperatures used. In addition, there is an increased hazard attendant upon handling this metal as it is very active chemically at the higher temperatures involved. Another disadvantage is that the time required to produce the superheating effect is relatively long and this immobilizes melting equipment which otherwise could be used for the production of molten metal for castings. Still another disadvantage is that the superheated metal, being so much hotter than generally desirable for making castings, must be cooled to a suitable casting temperature before pouring

2

into molds. This latter feature involves a further disadvantage in that the superheat effect rapidly disappears as the metal is cooled before casting so that the cooled superheat-treated metal must be poured into the molds soon after cooling if the grain refining effect of the superheating is to be retained.

I have now discovered that by subjecting the metal while in the molten state to a violent agitation (as distinguished from the ordinary stirring used in purification under a flux) by which the liquid metal undergoes intense shearing causing contiguous portions of liquid to slide over each other at a high rate, the grain size of castings made of the so-treated metal is greatly reduced, and, at least, the usual advantages of grain size reduction are obtained without many of the disadvantages of the superheating method heretofore used to reduce grain size. In particular, this result is obtained at a lower temperature and in less time than by the method heretofore known. As a consequence, less time is required to prepare the metal for making castings having a fine grain structure, less loss of metal occurs, consumption of flux, if used, is reduced, and the life of melting equipment is prolonged and its output increased.

The invention, then, consists of the method hereinafter fully described and particularly 30 pointed out in the claims, the annexed drawing and following description setting forth a mode of carrying out the invention and apparatus therefor.

In the drawings:

35 Fig. 1 is a side elevation largely in section of apparatus for maintaining and treating metal in the melted state in accordance with the invention.

Fig. 2 is an enlarged side elevation of a portion 40 of the apparatus of Fig. 1.

Fig. 3 is a plan view of the upper of the two apertured plates of the portion of the apparatus shown enlarged in Fig. 2.

Fig. 4 is a plan view of the lower of the two 45 apertured plates.

Fig. 5 is a view of the rotor attached to the lower end of the driving shaft shown enlarged in Fig. 2.

Fig. 6 is a modification of a portion of the apparatus of Fig. 1.

Fig. 7 is a sectional view on the line 7—7' of Fig. 6.

Fig. 8 is a fragmentary view of a portion of Fig. 6.

Throughout the drawings, like numerals refer to like parts.

As shown completely assembled in Fig. 1, the apparatus comprises a melting pot 1 mounted by its rim 2 in a furnace setting 3 provided with a heating burner 4 and flue 5. Resting on or attached to the rim 2 is a support in the form of a cover 6 having a charging port 7 with a removable cover 8. Passing through the cover 6 is a valved pipe connection 9 for controlling the passage of gas into or out of the space 10 above a body 11 of molten metal contained in the pot. The cover or support 6 also is provided with an opening 12 which supports the cover plate 13 on the upper side of which is mounted the agitator motor 14 and on the lower the agitator supports 15, which extend into the pot. In Figs. 1 and 2 attached to the lower ends 16 of the supports 15, there is shown the agitator baffle 17 of circular form and U-shape cross section. Within the baffle are upper and lower apertured plates 18 and 19, respectively. These are attached to the baffle at diametrically opposite points by the spacing bars 20. As shown, these plates are provided with concentric rows of small apertures 21 which may have a diameter of from about 0.125 inch to 0.562 inch, for example. For plates having a diameter of 7 inches, I have found that three equally radially spaced circular rows of apertures, 0.75 inch apart in the row, are satisfactory, although other arrangements and spacings may be used. These details are schematically shown in Figs. 3 and 4. Between the plates 18 and 19 operates the agitator rotor 22 attached to the lower end 23 of the drive shaft 24, the upper end of which is driven by the motor 14 through the shaft coupling 25. A bearing 26 supported by arms 27 attached to the supports 15 maintains the drive shaft in alignment. The upper apertured plate 18 is provided with a central opening 28 for admitting the drive shaft leaving a substantial annular opening between the drive shaft 24 and the adjacent edge of the plate. The lower plate 19 is also provided with a central opening 29, the area of which is preferably made substantially equal to that of the annular opening 28 so as to balance the liquid thrust which is developed when molten metal passes through these openings as the rotor revolves.

Again referring to the rotor 22, more particularly as shown in Fig. 5, the upper face 30 is provided with radial blades 31 extending a short distance, e. g. 1/4 inch, above the face of the rotor. The lower face is similarly provided with radial blades 32.

In the modification shown in Figs. 6, 7, and 8, the rotor and baffle have a modified form. As shown, the baffle comprises a pair of annuli, one designated 33 and the other 34. The annuli are supported by the lower ends 16 of the supports 15 and held in spaced relation with each other by a cylindrical screen 35 attached to the outer edges of the annuli. The screen may have small meshes, about 0.02 square inch in area being preferred, although other sizes may be used, e. g. from 0.01 square inch to 0.2 square inch in area.

Within the central openings 36 of the annuli operates the rotor 37. This consists of a plate member 38 attached to the lower end 23 of the drive shaft 24 and paddle blades 39 attached to the plate member.

In accordance with the invention, the metal to be treated is melted and its temperature raised to a suitable degree, the particular temperature employed being, in general, governed by the type of protective agent used over the metal, if any, e. g. flux, gas, etc., and while at such temperature, the molten metal is subjected to an intense shearing action as by a violent agitation in which contiguous segments of the molten metal are caused to move relatively to, or slide over, each other at a high rate. The rate of relative movement may be measured in terms of the ratio of the relative rate of movement of adjacent liquid metal segments to the distance between the segments. For convenience, this ratio may be referred to as the "shear gradient" or "velocity gradient" and may be expressed as velocity per unit distance of separation or per unit of gradient. Thus, the closer the segments the higher the velocity gradient for the same relative velocity of segments considered.

I have found that by subjecting contiguous segments of a body of the liquid metal to be treated to an intense shear in which a velocity gradient of about 30 feet per second or more per inch of metal thickness between the segments or per inch of gradient is produced, as by moving the liquid metal rapidly adjacent to a stationary surface which produces a frictional drag on the moving metal, the molten metal is sheared at a rapid rate and undergoes a change such that upon making a casting thereof the solid metal exhibits a finer grain structure in less treatment time than metal similarly melted and heated but not subjected to the aforesaid velocity gradient in the molten state. Only a few minutes is needed of the foregoing treatment to produce the grain refining effect in the usual size pot of the molten metal.

In order to facilitate carrying out the process of the invention in the foundry, for example, I have devised an apparatus, above described, in which the method may be practiced.

In carrying out the method with the apparatus illustrated in Figs. 1 to 5, inclusive, the magnesium-containing metal to be treated is introduced into the melting pot 1 through the opening 7 which is then closed with the cover 8 as shown. The metal is melted by heating the pot with the burner 4 and the temperature suitably raised. During melting and while the metal is in the molten condition, a suitable flux 40 may be employed over the metal to protect it from oxidation or a protective gas may be admitted through pipe 9 to contact the molten metal or both gas and flux may be used. The use of a protective inert gas, e. g. argon, helium, etc., has the advantage that the effect sought in the molten metal can be obtained at about 1200° F., although for best results a preferred operating temperature is 1250° F. If flux be used instead of such a gas but in the presence of air, the operating temperature must be raised to about 1350° F. or preferably to about 1400° F. However, if carbon monoxide or dioxide be substituted for the air, the operating temperature may be as low as 1200° F., the maximum safe working temperature with carbon dioxide and flux being about 1350° F. With inert gas alone, the operating temperature need not be so limited. In some

instances, it may be desirable to bubble the gaseous agent through the body of molten metal during treatment, as when the alloy involved is difficult to grain refine. For example, magnesium-base alloys containing between about 0.0005 to 0.1 per cent of beryllium are difficult to grain refine and may be treated advantageously by the combination of the violent agitation herein set forth and the bubbling of the gaseous agent through the melt. Other carbon-containing vaporizable materials may be used in place of carbon monoxide or dioxide, e. g.  $\text{CCl}_4$ ,  $\text{C}_2\text{H}_2$ , and  $\text{CH}_4$ .

After the metal has been heated to the proper temperature, the liquid metal is subjected to an intense shearing as by setting into rotation the rotor 22 of the agitator while submerged in the body of the metal, preferably maintained under a blanket of a flux or protective gas or both. As the rotor revolves, liquid metal is thereby induced to flow through the openings 28 and 29 and through the space between the faces of the rotor and the stationary plates 18 and 19. Liquid metal also passes through the openings 21 in the plates into the same space from which it is ejected by the action of the rotor aided by the sets of radial blades 31 and 32. The fast moving metal passing adjacent to the stationary plates is subjected to frictional drag by them and thereby has its velocity reduced as compared to the portions of the metal more remote from the stationary surfaces. A velocity gradient is thus set up in liquid metal as it traverses through the various openings and through the space between the rotor faces and the adjacent stationary plates producing shear, the magnitude of which is dependent upon the speed of rotation of the rotor.

With the apparatus shown (Figs. 1-5), the proper speed for operating the rotor can be calculated readily adopting as a basis the linear velocity of a point near the periphery of the rotor relative to the stationary plates 18 and 19. This basis is predicated on the fact that liquid metal adjacent to the rotor on traversing the spaces between the rotor 22 and adjacent plates 18 and 19 acquires a velocity relative to the adjacent stationary apertured plates substantially equal to that of the blades of the rotor at the periphery while the metal adjacent to the stationary plates tends to move slowly, if at all, due to frictional drag against these plates. For example, with a rotor of 7-inch diameter rotation at 1800 R. P. M. a point near the peripheral end of a blade travels at about 55 feet per second, and, if the clearance between the blades and the adjacent apertured plates be 0.25 inch, for example, then the velocity gradient is  $55 \div 0.25$ , i. e. 220 feet per second per inch. Such a velocity gradient is more than ample to produce the grain refining effect. The rotational speed of the rotor having a diameter of 7 inches and clearance of  $\frac{1}{4}$  inch sufficient to produce the desired effect is about 245 R. P. M.

After the metal has been subjected to the high shear or velocity gradient by causing it to traverse the space between the rotor and the adjacent stationary apertured plates, its lateral high velocity motion is abruptly modified, as by the baffle 17, so as to prevent violent turbulence but not circulation throughout the mass of molten metal not undergoing the shearing treatment. The arresting of the lateral motion or dissipation of the kinetic energy imparted to the molten metal by the rotor 22 in producing the violent turbulence, I have found, is generally necessary in order to prevent the beneficial effect of the treatment being undone. In this connection, I

have found, that if the treated metal is thereafter maintained under conditions permitting much general motion of the batch as a whole, grain refining effect of the high velocity gradient may be lost.

Essentially similar procedure is employed using the apparatus modified as in Figs. 6 and 7. With this form of apparatus the rotation of the rotor 37 causes a flow of metal through the meshes in the screen 35, as indicated by the arrows, and as a result both a high velocity gradient or shear is produced in each portion of the metal body which traverses the screen and the kinetic energy imparted to the metal is sufficiently dissipated to avoid loss of the grain refining effect obtained. The magnitude of the velocity gradient produced as the metal passes through the screen meshes is dependent at least upon the speed of rotation of the rotor and may be computed on the same basis as that already described for rotor 22. In this case, the linear velocity of the periphery of the rotor 37 divided by the spacing of the meshes in the screen is the velocity gradient. For example, with a 7-inch rotor rotating at 900 R. P. M., its linear velocity is 27.5 feet per second. Then, if the distance between the screen openings, i. e. the adjacent stationary surface is  $\frac{1}{8}$  inch, the velocity gradient is  $27.5 \div 0.125$  inch or 220 feet per second per inch.

The duration of the operation of producing a high shear gradient in the liquid so that all portions of a body thereof become so treated varies with the size of the body and the efficiency of the circulation through the device producing the velocity gradient. As an example, with the apparatus illustrated in a pot about 3 feet in diameter holding about 2000 pounds of metal, the time required is about 15 minutes.

The treated metal may be allowed to remain unused as long as about 30 minutes, or more in some cases, before the grain size of the castings made therefrom increases above that obtained upon casting the metal soon after the treatment. If the treated metal is allowed to remain unused long, it is advisable to retreat it as described before casting. If desired, the treatment may be continued, as by continuing the operation of the rotor, during the withdrawal of treated metal from the pot for casting.

With the form of apparatus illustrated, the agitator together with the driving motor can be lifted bodily off the cover of the melting pot and moved to other pots for treating baths of metal therein. And, while the agitator is thus removed, the treated metal may be readily ladled into molds, if desired.

The following examples are illustrative of the practice of the method.

#### EXAMPLE 1

A quantity of ingots weighing six hundred pounds consisting of "Dowmetal H," a magnesium-base alloy having a nominal composition of 6 per cent aluminum, 0.2 per cent manganese, and 3 per cent zinc, the balance being magnesium, was charged into a melting pot as in Fig. 1 and melted under a blanket 40 of flux (e. g. a mixture of 55 parts  $\text{KCl}$ , 34 parts  $\text{MgCl}_2$ , 9 parts  $\text{BaCl}_2$ , and 2 parts  $\text{CaF}_2$ ), air having access to the space 10 above the molten metal 11. The temperature of the molten metal was brought to  $1400^{\circ}$  F. and maintained at substantially this temperature in the ensuing treatment before which samples were removed and cast into test bars. These were sectioned, polished, and examined for grain size

which on the average was 0.023 inch in diameter. The molten metal in the pot was then subjected to a treatment to produce a velocity gradient in the metal above 30 feet per second per inch. This treatment was effected by the use of a rotor 7 inches in diameter, operating at 1800 R. P. M. between a pair of stationary plates spaced 0.5 inch from the rotor, a baffle similar to that shown at 17 being provided near the periphery of the rotor. The velocity gradient thus produced was computed to be 110 feet per second per inch of gradient, on the basis of the peripheral velocity of the rotor and the space between the faces of the rotor and the adjacent stationary plates. At one minute intervals during the treatment, samples of treated metal were removed, cast into test bars some of which were sectioned, polished, and examined for grain size, others were used for the determination of tensile strength properties. The data obtained are given below:

Table I

| Duration of Treatment, Minutes | Average Grain Size, Inches | Average Ultimate Tensile Strength, Lbs./sq. in. <sup>1</sup> | Average Yield Strength, Lbs./sq. in. <sup>1</sup> | Average Per Cent Elongation <sup>1</sup> |
|--------------------------------|----------------------------|--------------------------------------------------------------|---------------------------------------------------|------------------------------------------|
| 0                              | 0.023                      | 33,100                                                       | 11,000                                            | 9.3                                      |
| 1                              | 0.009                      |                                                              |                                                   |                                          |
| 4                              | 0.008                      |                                                              |                                                   |                                          |
| 5                              | 0.007                      |                                                              |                                                   |                                          |
| 6                              | 0.006                      |                                                              |                                                   |                                          |
| 9                              | 0.004                      |                                                              |                                                   |                                          |
| 13                             | 0.003                      |                                                              |                                                   |                                          |
| 15                             | 0.003                      | 40,500                                                       | 18,100                                            | 15.4                                     |
| 20                             | 0.003                      |                                                              |                                                   |                                          |
| 30                             | 0.004                      | 40,100                                                       | 12,900                                            | 15.1                                     |

<sup>1</sup> Properties measured after subjecting the test bars to conventional solution heat treatment.

## EXAMPLE 2

A batch of 60 pounds of Dowmetal H, containing about 0.0005 per cent of beryllium, was melted under a blanket of saline flux of the same composition as that in Example 1 and its temperature raised to 1250° F., an atmosphere of CO<sub>2</sub> being maintained above the melt. An agitating device of the form shown in Fig. 1 was submerged in the melt and the rotor revolved at a speed of from about 1000 R. P. M. to 1800 R. P. M. for 45 minutes. The batch was sampled and the samples cast into test specimens which were sectioned, polished, etched and examined for grain size with the following results:

Table II

| Duration of Treatment in Minutes<br>(before treatment) | Average Diameter of Grains in Inches |
|--------------------------------------------------------|--------------------------------------|
| 0                                                      | 0.010                                |
| 5                                                      | 0.005                                |
| 10                                                     | 0.006                                |
| 15                                                     | 0.005                                |
| 20                                                     | 0.002                                |
| 25                                                     | 0.004                                |
| 30                                                     | 0.003                                |
| 35                                                     | 0.004                                |
| 40                                                     | 0.002                                |
| 45                                                     | 0.0015                               |

The treatment has been used on many of the magnesium-base alloys among which are those containing from 4 to 10 per cent of aluminum and 0.1 to 0.3 per cent of manganese, either with or without zinc in amounts of 0.1 to 3.0 per cent, the balance being magnesium. Typical examples of common commercial alloys of the foregoing

type on which the process may be practiced are set forth in the table below:

Table III

| Dowmetal Alloy | Nominal Composition—Per Cent |     |            |            |
|----------------|------------------------------|-----|------------|------------|
|                | Al                           | Mn  | Zn         | Mg         |
| J-1            | 6.5                          | 0.2 | 1.0        | Remainder. |
| O-1            | 8.5                          | 0.2 | 0.5        | Do.        |
| C              | 9.0                          | 0.1 | 2.0        | Do.        |
| R              | 9.0                          | 0.2 | 0.6        | Do.        |
| G              | 10.0                         | 0.1 | Ca 0.1-0.2 | Do.        |
|                |                              | 2.0 |            |            |

15 In addition to the advantages aforementioned, the method has the further advantage of providing a way to reduce the grain size of the magnesium-base alloys containing beryllium which so far as known are not amenable to grain refinement by any conventional treatment.

I claim:

1. The method of grain refining prior to casting a molten magnesium-base alloy which comprises mechanically imparting to adjacent segments thereof a rapid relative motion and then substantially modifying their motion, said molten metal being maintained at a temperature between about 1200° F. and 1450° F., the method being performed without the introduction into the molten alloy of any carbonaceous material.

2. The method of grain refining prior to casting a molten magnesium-base alloy which comprises mechanically imparting to adjacent segments thereof a relative motion such that the relative velocity of the adjacent segments measured not over about 1 inch apart exceeds 30 feet per second and then substantially modifying their motion, said molten alloy being maintained at a temperature between about 1200° F. and

3. The method of grain refining prior to casting a molten magnesium-base alloy which comprises mechanically imparting to adjacent segments thereof a relative motion such that the relative velocity of the adjacent segments measured not over about 1 inch apart exceeds 30 feet per second and then substantially modifying their motion, said molten alloy being maintained at a temperature between about 1200° F. and 1450° F., the method being performed without the introduction into the molten alloy of any carbonaceous material.

4. The method of grain refining prior to casting a body of molten magnesium-base alloy which comprises maintaining a body thereof at a temperature between about 1200° F. and 1450° F., continuously withdrawing molten metal from the body and mechanically ejecting it through a fine mesh screen submerged in the body of the molten metal whereby the molten metal traversing the screen meshes undergoes a violent shearing effect, the method being performed without the introduction into the molten alloy of any carbonaceous material.

5. The method of grain refining prior to casting a body of a molten magnesium-base alloy which comprises submerging a fluid pump therein, said pump being provided with a screen over its discharge opening, said screen being submerged in the molten metal and operating the fluid pump so as to withdraw molten metal from the body thereof and drive it through the meshes in the screen, the said molten body of alloy being maintained at a temperature between about

75

2,472,757

9

1200° F. and 1450° F., whereby the molten metal traversing the screen meshes undergoes a violent shearing effect, the method being performed without the introduction into the molten alloy of any carbonaceous material.

6. A method of grain refining aluminum magnesium casting alloys including mechanically agitating a body of the molten alloy while at a temperature of approximately 1400° F. just prior to casting, and without the introduction there-  
into of any carbonaceous material.

JOHN S. PEAKE.

## REFERENCES CITED

The following references are of record in the 15 file of this patent:

10

## UNITED STATES PATENTS

| Number    | Name          | Date          |
|-----------|---------------|---------------|
| 1,555,956 | Bakken        | Oct. 6, 1925  |
| 2,066,579 | Schichtel     | Jan. 5, 1937  |
| 2,195,092 | Muller et al. | Mar. 26, 1940 |
| 2,275,266 | Meyer         | Mar. 3, 1942  |
| 2,380,863 | Nelson et al. | July 31, 1945 |

## OTHER REFERENCES

10 Hultgren et al., University of California, Final Advisory Report to the War Production Board; Report No. W-147, W. P. B. Research Project NRC-550 on "Control of Grain Structure and its Effect on Quality of Magnesium Alloy Castings," April 23, 1946, 4 pp. Preface and pages 9, 19, 42, 43 and 44.